

Jan. 27, 1970

C. R. SHEEHAN ET AL

3,492,144

METHOD OF MAKING FLOCKED FABRICS

Filed Feb. 1, 1966

2 Sheets-Sheet 1



Fig. 1



Fig. 2



Fig. 3



Fig. 4



Fig. 5

INVENTORS  
Charles R. Sheehan  
BY Paul McDowell

*N. Elliott Dry*

ATTORNEY

Jan. 27, 1970

C. R. SHEEHAN ET AL

3,492,144

METHOD OF MAKING FLOCKED FABRICS

Filed Feb. 1, 1966

2 Sheets-Sheet 2



Fig. 6



Fig. 7

INVENTORS.  
Charles R. Sheehan  
BY Paul McDowell

*Y. Elton Dry*

ATTORNEY

1

3,492,144

**METHOD OF MAKING FLOCKED FABRICS**  
Charles R. Sheehan, Williamsburg, and Paul McDowell,  
Newport News, Va., assignor to The Dow Chemical  
Company, Midland, Mich., a corporation of Delaware

Filed Feb. 1, 1966, Ser. No. 524,142

Int. Cl. B44c 1/08

U.S. CL. 117—33

2 Claims

## ABSTRACT OF THE DISCLOSURE

This invention discloses and claims an improved method for making a flocked fabric which method comprises curling relatively long sections of synthetic polymer filaments and thereafter applying the curled sections of filament to an adhesive coated fabric backing material.

This invention relates to flocked fabrics and a novel method of making same. More particularly, the invention relates to flocked fabrics that are made from long, curled sections of synthetic monofilament, which exhibit improved wear, pile resiliency, and general appearance.

Flocking is of great importance as a modern method of surface styling for textiles and plastics. In this surface treatment, natural or synthetic dust, short fibers of different staple length and denier, or flocks of definite length and diameter are cemented by a bonding agent to the entire surface or part of it, of textiles, non-wovens, or plastic or metal foils, and also to leather, rubber, wood, paper, glass and sheet metal. Hence flocked material always consists of basic material, bonding agent and pile.

One of the basic difficulties in the flocking art is the ability to obtain a dense, resilient flocked carpet using relatively long, cut fibers. Generally, when longer fibers are used, both flock density and orientation are poor. This is particularly true with acrylic, polyolefin and vinylidene chloride-vinyl chloride polymer fibers. Due to their resistance to the elements, these fibers are ideal for outdoor carpet and decorative coverings. However, it has been necessary to resort to tufted-type coverings and carpet to obtain a product that is acceptable.

Tufting with these materials still does not solve the problem of resiliency and appearance. The fibers tend to lay flat and fail to present a fresh appearance after even limited use.

In order to overcome these and related disadvantages, it has been discovered that flocked fabrics, having improved wear, pile resiliency and appearance, can be produced by a method which comprises curling relatively long sections of thermoplastic monofilaments and then applying the curled sections of monofilament to an adhesive coated suitable fabric backing material.

Flocked fabrics produced in this manner possess a pile density, resilience, durability and attractive appearance that are novel to the flocked fabric art.

The present invention will be more readily apparent and easily understood by reference to the ensuing disclosure and specification taken together with figures of the drawings, in which:

FIGURE 1 is a fragmentary transverse sectional view of a flocked fabric made using straight, non-curved filament sections;

FIGURE 2 is a fragmentary transverse sectional view of a flocked fabric made in accordance with the invention using curved filament sections;

FIGURE 3 is a perspective view of a flocked fabric made using straight, non-curved filament sections;

FIGURE 4 is a perspective view of a flocked fabric of the present invention using curved filament sections;

2

FIGURE 5 is a transverse view of individual filament sections possessing varying degrees of curl;

FIGURE 6 is a schematic view of a mechanical process employed for manufacturing the flocked fabrics of the invention; and

FIGURE 7 is a schematic view of an electrostatic process employed for manufacturing the flocked fabrics of the invention.

Referring now to the drawings and as may be best seen in FIGURE 1, flocked fabrics having relatively long, straight filament sections 12 tend to be flat on the fabric surface 10. In addition, there is poor covering and density, yielding a fabric that is both unsightly and unacceptable in the market place. However, in FIGURE 2, there is illustrated the remarkable advantages of using a filament section 13 in flocking a fabric. Depending on degree of curl and length of filament section, a great degree of resiliency and fiber density can be tailored into the finished flocked fabric.

The perspective view of FIGURE 3 and FIGURE 4 more clearly illustrate the unexpected result of pile density and resiliency built into the flocked fabric using curled filaments. FIGURE 3 illustrates the poor covering of straight, non-curved filaments and shows their tendency to lie down on the fabric backing rather than standing perpendicular. This effect is well known in the art and is the main reason long filaments are generally omitted from most flocking methods.

In contrast to the inadequate fabric of FIGURE 3, is the flocked fabric illustrated in FIGURE 4, wherein curled filaments comprise the pile surface of the fabric. It can be seen readily that the curled fabrics tend to interlock, causing a much greater resiliency and density than is normally found in flocked fabrics using long filaments.

The filament sections useful for the present invention have a length of from about  $\frac{1}{4}$  to  $1\frac{1}{2}$  inch and are preferably in the range of 15 to 1250 denier, depending on choice of polymer filament. The degree, or amount, of curl is illustrated in FIGURE 5 wherein the individual filament sections are shown possessing varying curl. The degree of curling was established using a  $\frac{1}{2}$  inch cut flock and measuring the radii of curvatures, which preferably run from  $\frac{1}{16}$  to  $\frac{5}{16}$  inch. This can be better understood by referring to FIGURE 5e, wherein the dotted line, defining the chord, is a measure of the radius of curvature. It can be seen readily that FIGURE 5a would of course, be  $\frac{1}{16}$  inch curvature, with FIGURE 5f being  $\frac{5}{16}$  inch curvature. FIGURE 5b has  $\frac{1}{16}$  inch curvature, 5c having  $\frac{1}{16}$  inch curvature, and so forth. There is a variance in desirable degree of curl, depending on the particular properties desired in any given flocked fabric. For this reason, FIGURE 5 is merely for purposes of illustration and is not to be construed as limiting the invention herein.

Referring now to FIGURE 6, there is illustrated schematically one method of manufacturing the flocked fabrics of the present invention. The method consists essentially of passing a suitable fabric material 16 onto a conveyor 24, where a suitable adhesive 19 is uniformly coated onto fabric 16 and smoothed by a doctor blade 28. The adhesive-coated fabric 20 is then conveyed beneath a flock distributing device 26 which drops the cut filament sections 25 onto the coated fabric 20. To drive the filament sections 25 into the adhesive 19 and to increase the pile density, rotation beater bars 23, located beneath the conveyor 24, vibrate the coated fabric 20, tending to drive the coated fabric 20 upward as the flock 25 falls downward. There is preferably a pneumatic force applied subsequently to the flocked fabric 30 by a pneumatic device 27 so as to remove excess loose flock from the finished

fabric. The finished fabric 30 is then conveyed on to subsequent drying and like treatments.

FIGURE 7 illustrates an alternative method employing electrostatic flocking, as opposed to mechanical flocking of FIGURE 6. As can be seen, the essential steps are the same as in FIGURE 6, except there is now a positive electrode grid 31 through which the curled flock 25' is dropped, onto the moving adhesive-coated fabric 20', from the flock hopper 26'. There is located beneath the coated fabric 20' a grounded electrode 29. As the curled flock 25' passes through grid 31, the flock becomes charged and is "fired" into the adhesive coating 19, with flock 25' that does not stick reversing their charge and being fired back to grid 31, where the flock 25' again reversing polarity and being fired back to the adhesive-coated fabric 20'. This action occurs rapidly until the flocked fabric 30' passes beyond the grids 29 and 31. Preferably, excess flock is pneumatically removed by a suction device 27' following the flocking operation.

There are many suitable adhesives available commercially, with the acrylic-type adhesives being preferred due to their weather resistance and relatively long pot life.

The present invention can be practiced with most synthetic filaments available. Preferably, the filamentary material is a vinylidene chloride-vinyl chloride copolymer (Saran Flat Microtape) of about 400 denier. Filaments of polypropylene, polyethylene, nylon, polyesters, acrylates, and vinyl of from 15 to 600 denier are also well adapted for use in the invention.

There are many ways to curl thermoplastic filament sections, such as by treating with hot air, steam and hot water with or without mechanical agitation. It has been found that treatment in hot air at about 225° to 275° F. for about 2-10 minutes produces a suitable curl. Steam treatment at atmospheric pressure for about 15 to 30 seconds is equally suitable. Equally good results are obtained by treating the filaments in water at about 200° to 210° F. for about 5 minutes if the flock is predyed at about 210° F. for 60 minutes. Variations in temperature and time can be made to obtain the desired degree of curl for

This was flocked onto a 225 square inch sample of woven SFM, and coated with 16 ounce per square yard of acrylic adhesive, as in Example 1, above. Flock in the amount of 2.14 grams was retained on the backing. The density of flock on the sample was 12.3 ounce per square yard, showing approximately a 100 percent increase in flock density resulting from the use of pre-curved flock.

### EXAMPLES 3-9

Various heat treatments were tried using 400 denier SFM,  $\frac{1}{2}$  inch cut, and subsequently applied to adhesive-coated fabric pieces. In each batch of cut flock there was a distribution of degree of curling. Set out below is Table I showing the heat treatment and distribution of curling. The data makes abundantly clear the relatively wide variance in acceptable heat treatments applicable for the present invention. (Examples 3-7 were conducted with hot air.)

TABLE I.—DISTRIBUTION OF CURLING OF SFM

| Heat treatments               | Degree of curl percent |       |       |       |       |
|-------------------------------|------------------------|-------|-------|-------|-------|
|                               | 2/16"                  | 3/16" | 4/16" | 6/16" | 8/16" |
| (3) 250° F., 5 minutes        | 2                      | 10    | 18    | 60    | 10    |
| (4) 275° F., 5 minutes        | 13                     | 17    | 38    | 32    | —     |
| (5) 300° F., 5 minutes        | 5                      | 45    | 35    | 15    | —     |
| (6) 275° F., 2 minutes        | 4                      | 10    | 10    | 36    | 40    |
| (7) 275° F., 10 minutes       | 5                      | 50    | 35    | 10    | —     |
| (8) Boiling water, 10 minutes | 5                      | 70    | 25    | —     | —     |
| (9) Boiling water, 10 minutes | 5                      | 55    | 25    | 15    | —     |
| Dry at 250° F.                | 5                      | 55    | 25    | 15    | —     |

### EXAMPLES 10-22

Flocked fabrics were prepared in the manner of Example 1 using fibers of vinylidene chloride-vinyl chloride (Saran Flat Monofilament), polypropylene, polyamide, metal (coated with thermoplastic such as Lurex manufactured by The Dow Chemical Company), polyester, and acrylic. The flocked fabrics were inspected to determine the number of pile fibers per square inch. Samples were made with both curled and non-curved to demonstrate the greater fiber density of the curled flock over the non-curved flock. Table II, below, contains the results of the experiment.

TABLE II

| Sample No. | Class of Fiber | Type      | Dimensions           | Denier | Flock          |               | File Flock Test Data |                       |                      |                       |
|------------|----------------|-----------|----------------------|--------|----------------|---------------|----------------------|-----------------------|----------------------|-----------------------|
|            |                |           |                      |        | Degree of Curl | Length of Cut | Curled               | Not Curled            |                      |                       |
|            |                |           |                      |        | Radius (in.)   | (in.)         | Oz./yd. <sup>2</sup> | No. of Fibers sq. in. | Oz./yd. <sup>2</sup> | No. of Fibers sq. in. |
| 10         | Saran          | Microtape | 3 mils x 25 mils     | 400    | 0              | 8/16          | —                    | —                     | 4.2                  | 20                    |
| 11         | do             | dop       | do                   | 400    | 2/16           | 8/16          | 11.2                 | 402                   | 4.2                  | 20                    |
| 12         | do             | do        | do                   | 400    | 3/16           | 8/16          | 10.7                 | 388                   | 4.2                  | 20                    |
| 13         | do             | do        | do                   | 400    | 4/16           | 8/16          | 10.3                 | 360                   | 4.2                  | 20                    |
| 14         | do             | do        | do                   | 400    | 6/16           | 8/16          | 10.0                 | 305                   | 4.2                  | 20                    |
| 15         | do             | do        | do                   | 400    | 8/16           | 8/16          | 7.8                  | 191                   | 4.2                  | 20                    |
| 16         | Polypropylene  | do        | 3.3 mils x 18.6 mils | 225    | 4/16           | 8/16          | —                    | 321                   | —                    | 98                    |
| 17         | do             | Oval      | 6.6 mils x 21.1 mils | 575    | 4/16           | 8/16          | —                    | 228                   | —                    | 128                   |
| 18         | do             | Round     | Diameter 2.0 mils    | 14.3   | 4/16           | 8/16          | —                    | 1,285                 | —                    | 149                   |
| 19         | Polyamide      | Trilobal  | 2.1 mils             | 15     | 4/16           | 8/16          | —                    | 1,696                 | —                    | 104                   |
| 20         | Metallic       | Slit Film | 1 mil x 10 mils      | 110    | 4/16           | 8/16          | —                    | 700                   | —                    | 5                     |
| 21         | Polyester      | do        | 1 mil x 10 mils      | 76     | 4/16           | 8/16          | —                    | 874                   | —                    | 68                    |
| 22         | Acrylic        | Round     | Diameter 3.1 mils    | 32.5   | 4/16           | 8/16          | —                    | 1,044                 | —                    | 710                   |

a given polymer filament section without departing from the spirit or scope of the present invention.

### EXAMPLE 1

Five grams of 400 denier Saran flat microtape (SFM)  $\frac{1}{2}$  inch, precision cut flock was applied using a laboratory mechanical flocking machine to a 225 square inch sample of woven SFM fabric coated with 16 ounce per square yard of acrylic adhesive.

After mechanical beating, 1.08 grams of flock was retained on the adhesive backing. This resulted in a flock density of 6.2 ounce per square yard. Cover was extremely poor; resiliency was nil.

### EXAMPLE 2

Five grams of the same 400 denier SFM  $\frac{1}{2}$  inch cut was pre-curved by hot water at 210° F. for 60 minutes.

The above results clearly show that the curling, of the present invention, results in an increase in pile density of from 47 to several thousand percent. In addition, the interlocking action of the curled fibers in the finished fabric cause a greater resiliency in the fabric than heretofore known.

We claim:

1. A method of producing wear and weather resistant flocked fabrics which comprises curling relatively long sections of synthetic polymer filaments into arcuate segments and thereafter applying the arcuate segments of filament to an adhesive coated suitable fabric backing material.

2. The method of claim 1 wherein the synthetic polymer is a thermoplastic.

(References on following page)

## References Cited

## UNITED STATES PATENTS

|           |         |               |           |
|-----------|---------|---------------|-----------|
| 2,326,174 | 8/1943  | Rutishauser   | 19—66 X   |
| 2,377,810 | 6/1945  | Robbins       | 264—168   |
| 2,439,815 | 4/1948  | Sisson        | 161—177   |
| 2,917,806 | 12/1959 | Spence et al. | 264—168 X |
| 3,322,606 | 5/1967  | Koller        | 161—64 X  |
| 3,330,896 | 7/1967  | Fujita et al. | 264—168 X |

5

|           |         |           |        |
|-----------|---------|-----------|--------|
| 1,939,846 | 12/1933 | Fenton    | 117—33 |
| 1,949,068 | 2/1934  | Achterhof | 117—28 |
| 3,024,518 | 3/1962  | Newton    | 161—66 |
| 3,275,487 | 9/1966  | Lemelson  | 156—72 |
| 3,314,845 | 4/1967  | Perri     | 161—64 |

WILLIAM D. MARTIN, Primary Examiner

U.S. Cl. X.R.

117—17, 20